

F. G. KEYES & R. B. BROWNLEE.  
PRODUCTION OF METALLIC TUNGSTEN.  
APPLICATION FILED JULY 6, 1914.

Patented Oct. 24, 1916.

1,202,534.



WITNESSES

Chas. Clagett  
Thos. H. Brown

INVENTORS  
Frederick G. Keyes  
Robert B. Brownlee  
BY  
George H. Stockwell  
ATTORNEY

# UNITED STATES PATENT OFFICE.

FREDERICK G. KEYES AND ROBERT B. BROWNLEE, OF EAST ORANGE, NEW JERSEY,  
ASSIGNEES TO COOPER HEWITT ELECTRIC COMPANY, OF HOBOKEN, NEW JERSEY,  
A CORPORATION OF NEW JERSEY.

## PRODUCTION OF METALLIC TUNGSTEN.

Specification of Letters Patent.

Patented Oct. 24, 1916.

1,202,534.

Application filed July 6, 1914. Serial No. 849,137.

*To all whom it may concern:*

Be it known that we, FREDERICK G. KEYES and ROBERT B. BROWNLEE, citizens of the United States, and residents of East Orange, 5 county of Essex, State of New Jersey, have invented certain new and useful Improvements in the Production of Metallic Tungsten, of which the following is a specification.

10 The attempt to produce metallic tungsten by electrolytic processes has hitherto shown very meager results. It has been found, for example, that it is impossible to obtain tungsten electrolytically from an aqueous 15 solution of its salts. It has also been found that only the so-called tungsten-bronzes can be obtained from molten para-tungstates. Moreover, while we have found that tungsten tri-oxid gives a clear solution in boric 20 acid at 1000 to 1200 degrees centigrade, even with a high concentration of the tri-oxid, yet such a solution submitted to a tension of from 110 to 500 volts at temperatures from 1000 to 1300 degrees centigrade permits 25 only a fraction of an ampere to pass. Separation of tungsten took place when the electrolytic action was prolonged, but the process was necessarily slow and, for that reason, was temporarily cast aside. Similar 30 results were obtained with a solution of tungsten oxy-chlorid in fused boric acid. A practical process of producing metallic tungsten is found, however, by igniting for a more or less prolonged period  $WO_3$  at 35 1800 to 2000 degrees C. Under these conditions the liberation of oxygen takes place, resulting in the formation of lower oxids of tungsten and the production of a dark blue crystalline substance which conducts electricity 40 readily at ordinary temperatures. The substance is fluid at about 2000 degrees centigrade and in its fluid condition may be utilized as an electrolytic bath from which metallic tungsten can be separated by the 45 servance of a proper mode of procedure.

In general we prefer to employ a rotating cathode of tungsten and an anode in the form of a sintered rod of tungsten, through which and through the oxid bath an electric 50 current is passed. Varying current densities may be employed according to the char-

acter of the deposit desired, the dimensions of the bath, the volume of the electrolyzing fluid, and the area of the electrodes. The crucible itself should be of tungsten or high 55 melting alloy of tungsten; that is, it should be of such a character as not to contaminate the bath with impurities if it is desired to produce pure tungsten. If, however, it be desired to produce, for example, a carbon- 60 bearing deposit, the crucible material may contain carbon.

In order to bring the electrolytic substance into a fluid condition, and to maintain it in such condition during the electrolyzing process, use is made of the fact that the substance conducts electricity when cold and may consequently carry current enough to bring it to a fluid condition through the action of the  $I^2R$  heat or Joule heat. As 70 suming that the lower oxid formed by the initial ignition above referred to is  $WO_2$ , we know that the heat of formation of this oxid is 131,000 calories per gram molecule; hence, about one volt is the decomposition or deposition potential. Sufficient energy in addition to this must be applied to maintain the 75 material in a fluid condition.

Recapitulating the foregoing description of the novel process herein described, the 80 steps consist, first, of a more or less prolonged ignition of  $WO_3$ , at 1800 to 2000 degrees centigrade. This results in the liberation of a portion of the oxygen, leaving a lower oxygen compound or a mixture of 85 such oxygen compounds. Thus, the first step in the process may leave  $WO_2$  or  $WO$  or a mixture of these two oxids. The substance resulting from this part of the process is then brought to a fluid state and maintained in said state, preferably by means of 90 the  $I^2R$  heat, and a surplus of energy is applied to the material for maintaining it in a fluid condition. The application of electric current to this fluid material causes a compact deposit of metallic tungsten upon the 95 cathode. As already stated, the cathode is of tungsten, and preferably a rotating cathode, while the anode is, for example, a tungsten anode consisting of a sintered rod of 10 tungsten. The density of the current applied to the bath varies according to condi-

- tions already stated. It has been found that at high temperatures anodes of high melting metals, as iridium, become oxidized at the anode in this bath since oxygen is liberated, and that, moreover, such oxid passing into the solution, the metal ion is deposited upon the cathode, thereby producing an alloy, or at any rate, contaminating the deposit of pure tungsten which it is desired to obtain.
- 10 Of course, an ideal electrode would consist of a cast bar of lower tungsten oxids since they conduct the electric current with facility. As a matter of course, the melting point of such an oxid would be the same as the bath in which the electrolysis is being carried out and hence the use of such an anode is precluded. The melting point of the anode, however, may be adjusted by mixing the lower tungsten oxid and tungsten powder and casting this into the form of an anode bar. Obviously, such an anode or, at least the particles of tungsten composing it, will be attacked by the anion, in the present instance oxygen, forming oxid in all probability and thereby becoming a portion of the bath itself. This is desirable and forms as will be readily perceived, a means of renewing the electrolytic bath.
- 15 Other anodes, of course, may be used depending upon the character of the cathode deposit desired.
- It is convenient to use as the cathode a tungsten wire about one-sixteenth of an inch in diameter. The first wire used in the formation of subsequent tungsten wires may be of iridium, for example, and after a deposit of considerable thickness of metallic tungsten has been formed upon this iridium wire the ingot thus created may be swaged down and a part of the resulting wire again used as a cathode. By repeating this process the iridium is finally eliminated and a pure tungsten wire to form the cathode is obtained.
- 20 It will be understood that we have mentioned the use of an original iridium cathode simply to explain how we may produce subsequent materials for cathodes which are made in accordance with the herein described process. After the iridium has been removed by repeated operations such as have been described, wires or other shapes of our grade or quality of tungsten may be utilized as cathodes. There is, of course, no controlling reason why ordinary commercial tungsten should not constitute the cathode, if desired or if suited to special needs or requirements. When sufficient tungsten has been deposited upon the cathode, the wire may be removed and another substituted. In practice, to prevent the bath from cooling, it is recommended to use two rotating cathodes, one of which may be removed and a new cathode placed in the electrode holder. The electrode, with its tungsten deposit, is then swaged down to a diameter where it is practical to reduce the diameter still further by drawing dies.
- 25 Plainly, the process described herein may be utilized for refining a metal or for obtaining a metal from its soluble salts. There is no distinction, so far as the nature of the process goes. The case of tungsten, if that be the metal sought to be thrown down by the present process, is completely analogous to the well-known copper process, wherein copper is obtained from its soluble salts by using a magnetic anode or a platinum anode in a solution of copper or wherein an electrolytic refining of copper is obtained by means of an impure copper bar used as an anode.
- 30 For certain purposes it is desirable to obtain very pure tungsten and to this end bars pressed up from partially reduced tungstic trioxide may be utilized as anodes. It is obvious that a pressed bar, even of pure metal, would not be homogeneous, whereas an electrolytically disposed metal would of necessity be homogeneous. It would be possible to use a pressed bar of  $WO_3$ , which has a sufficiently high melting point but it is more convenient to reduce tungsten trioxide to the point where it contains enough lower oxide to increase the melting point above the temperature at which it is to be used as an anode. Usually, in this case, a small amount of metal will be present in the resulting powder. It is, of course, possible to reduce tungsten with carbon in the electric furnace, and press and sinter this material into bars which will serve as anodes. In any electrolytic process, for every equivalent of electrochemical material deposited upon the cathode, the same electrochemical equivalent must be taken from the bath or from the anode.
- 35 In the foregoing specification we have stated that it is desirable that the cathode be caused to rotate. The object of this scarcely requires explanation, but it will be understood that the rotation of the cathode will cause a more even deposit of tungsten upon the cathode element and that the same act of rotation will tend to keep the bath in an active condition with a more or less free circulation of the bath liquid.
- 40 We have illustrated the means for rotating the cathode in the accompanying drawing which is a vertical section of a tubular furnace containing a crucible within which are located the anode and the cathode of the system.
- 45 The furnace itself is shown at 1 and the crucible inside the furnace at 2. Within the crucible is the electrolytic bath 3 already described. The crucible is subjected to very high temperature and must be of very refractory material, preferably tungsten. It is not necessary that the crucible be made of

pure tungsten, although the material employed for the crucible should be such as would not contaminate the bath contained in it. A support 4 sustains the crucible as shown.

5 The anode of the bath appears at 5, and the cathode at 6. Both are connected by an electric circuit, the opposite terminals of which run to a storage battery 7.

10 It has been stated that it was of advantage to have the cathode rotate during operation. This is accomplished by means of a pulley having a V shaped groove and a bearing, together with an independent operating 15 driving motor. The bearing is shown at 8, the pulley at 9, and the driving motor at 10, the pulley and driving motor being connected by a band 11. Because of the high temperature of the bath, it is preferable to 20 mount this pulley bearing and the driving mechanism therefor at a point well removed from the surface of the crucible.

25 As to the details of the furnace, the same is preferably made of graphite and is provided with enlargements 12 and 13, through which connection is made to the terminals of the transformer, either with or without the intervention of bands 14 and 15 of metal or other conductor surrounding the enlargements.

30 The primary of the transformer forming the direct means for energizing the furnace, is shown at 16 and four coils 17, 17, arranged in parallel, constitute the secondary of the 35 primary 16, and are connected to the furnace

at 14 and 15. The drawing shows practically the entire system described herein.

We claim as our invention:

1. The method of producing pure tungsten which consists in bringing an oxid of tungsten to a fluid condition in an inert environment, maintaining the said condition by Joule heat, and separating the tungsten from the electrolyzing bath by an electrolytic process.

40 2. The method of separating metallic tungsten which consists in subjecting tungsten trioxid to a temperature of approximately 2000 degrees centigrade, thereby producing a lower oxid or mixture of oxids conductive of electricity and also thereby bringing the resultant substance to a fluid condition, maintaining such a condition and passing an electric current therethrough.

45 3. An electrolytic apparatus comprising a bath of fluid oxid of tungsten, a rotating tungsten cathode and a highly refractory anode.

50 4. In a fused electrolyzing bath, a cathode of pure tungsten and an anode consisting of a sintered rod of pure tungsten.

55 Signed at New York in the county of New York and State of New York this 3rd day of July, A. D. 1914.

FREDERICK G. KEYES.  
ROBT. B. BROWNLEE.

Witnesses:

GEORGE H. STOCKBRIDGE,  
THOS. W. BROWN.